

938,352.

E. R. TAYLOR.  
ART OF ELECTRIC SMELTING.  
APPLICATION FILED MAR. 3, 1909.

Patented Oct. 26, 1909.

4 SHEETS—SHEET 1.

FIG. 1.



E. R. TAYLOR.

ART OF ELECTRIC SMELTING.  
APPLICATION FILED MAR. 3, 1909.

938,352.

Patented Oct. 26, 1909.

4 SHEETS—SHEET 2.

Fig. 2.



### Inventor

## Witnesses

W. St. Evans.

M. E. Snod

20  
10  
P.P. Edward R. Taylor

May 20th 1901

Attorney

E. R. TAYLOR.  
ART OF ELECTRIC SMELTING.  
APPLICATION FILED MAR. 3, 1909.

938,352.

Patented Oct. 26, 1909.

4 SHEETS—SHEET 3.

*Fig. 3.*



*Fig. 4.*



Witnesses

H. S. Durang

M. E. Snell

Edward R. Taylor

Edward R. Taylor

Attorney

938,352.

E. R. TAYLOR.  
ART OF ELECTRIC SMELTING.  
APPLICATION FILED MAR. 8, 1909.

Patented Oct. 26, 1909.

4 SHEETS—SHEET 4.

Fig. 5.



Fig. 6.



Fig. 7.



Inventor

Witnesses

W. M. Barnes.

M. E. Smoot

Edward R. Taylor

+ by

R. E. Swan,

Attorney

# UNITED STATES PATENT OFFICE.

EDWARD R. TAYLOR, OF PENN YAN, NEW YORK.

## ART OF ELECTRIC SMELTING.

938,352.

Specification of Letters Patent.

Patented Oct. 26, 1909.

Original application filed June 12, 1908, Serial No. 438,115. Divided and this application filed March 3, 1909.  
Serial No. 481,121.

*To all whom it may concern:*

Be it known that I, EDWARD R. TAYLOR, a citizen of the United States of America, and a resident of Penn Yan, in the State of New York, have invented a new and useful Improvement in the Art of Electric Smelting, of which the following is a specification.

This invention relates primarily to the electric smelting of oxid iron ores by a continuous process; but novel features of the process may be used for effecting other reactions and reductions.

The present invention consists in the improved process of smelting oxid iron ore or similar metallurgical material in an electric furnace hereinafter described, and certain novel features thereof, as more particularly set forth in the claims hereto appended.

The invention is in part additional to the "Improvement in the art of producing chemicals in electric furnaces" set forth in my specification forming part of United States Letters Patent No. 702,117, dated June 10, 1902.

The objects of the present invention common thereto and to said patented improvement include the protection of horizontal or substantially horizontal electrodes against excessive wear, and the regulation of the electric action within the furnace, by means of fragmentary conducting or resistance regulating material, fed by gravity upon said electrodes and between the same; the interception and utilization to the utmost of heat that would otherwise be lost by radiation; and the avoidance of the cooling of the more highly heated inner part of the furnace or heat zone, in continuous reactions and reductions, by the sudden introduction of cold material, so as to insure the continuity of the operation.

Other objects common to said patented improvement and the present invention are to utilize in an effective manner the alternating or two-phase electric current, and to provide for varying the paths of the electricity through the charge within the working chamber so as to prevent the formation of piers of the less fusible ingredients of the charge or to burn out such piers should they accidentally be formed.

Other objects, including most of those hereinafter stated, are common to the present improvement and to my improvement in "electric smelting furnaces" more particu-

larly described and claimed in the specification forming part of my application for patent filed June 12, 1908, Serial No. 438,115; the application for patent of which my present specification forms part, being a required division of said application Serial No. 438,115.

The leading object is to overcome certain difficulties that present themselves in the electric smelting of metals and other electrically conductive materials in a shaft furnace, and especially to keep the material of the charge between the electrodes from becoming so conductive of electricity as to reduce the resistance of the furnace below practicable working limits.

Other objects are the separation of the ore in the four quarters of a two-phase furnace having two pairs of horizontal or inclined main electrodes, hereinafter referred to in common as "horizontal", arranged in vertical planes at right angles to each other, so as to keep the same separate, and thus to facilitate the manipulation of the ore within the furnace; to provide for employing a large proportion of fine ore, such as cannot be smelted in a blast furnace because of its liability to be blown out of the furnace by the blast; to provide for feeding fine and coarse ore downward in a stack furnace in separate vertical or substantially vertical columns; to utilize a portion of the charge and especially the fine ore columns for the conservation of the heat of the furnace, by feeding the same downward at or near the periphery of the furnace to a suitable point above horizontal main electrodes, and there feeding the same inward by a stoking operation to so regulate the feed of such material as to properly utilize the energy liberated between the main electrodes without causing short circuits; to provide for admitting successive small quantities of fine ore into the outer edges of the coarse ore columns in order to gradually bring the hottest of the fine ore in toward the center of the furnace, and to relieve the stress of stoking to that extent; to provide for feeding suitable carbonaceous material, preferably either coke or charcoal, in a central column, and for utilizing lateral wings of such "coke column," as it is hereinafter termed, to separate the columns of coarse ore; to utilize such coke column as a resistance conductor between secondary electrodes located at the

39

65

70

75

80

85

90

95

100

105

110

bottom and top of the furnace respectively; to provide in this way for starting the furnace with facility by the interaction of said secondary electrodes and said coke column; 5 to keep the carbonaceous material of the charge incandescent to a greater height than has heretofore been practicable; to vary the height of such incandescence at will; to determine thus the percentage of carbon, for 10 example, in the reduction of iron, so as to produce pig iron or steel as may be desired; to insure the reduction of ore to metal, to as considerable an extent as may be possible, in the fine ore before it reaches the heat zone, 15 and to utilize the heat between said horizontal electrodes for superheating the streams or globules of fluid metal as they trickle downward, so that they shall carry with them into the hearth sufficient heat to 20 keep the metal in the hearth in a fluid condition.

Another object of the invention is to oxidize accumulations of carbon or other oxidizable materials which may at times form 25 to an undesirable amount and interfere with the regular working of the furnace.

Other objects peculiar to the present improvement and said companion improvement in electric smelting furnaces relate especially to the production in an electric 30 furnace of iron or steel, hereinafter referred to in common as metal, from iron ores consisting of or containing sesquioxid of iron,  $Fe_2O_3$ , or magnetic oxid,  $Fe_3O_4$ , or 35 other forms of iron oxid adapted for like treatment. Sesquioxid of iron, for example, at a sufficient but low temperature, in contact with carbonic oxid gas also at a low but sufficiently high temperature, undergoes substantially the following reaction, that is to 40 say:  $1(Fe_2O_3) + 3(CO) = 2Fe + 3(CO_2)$ .

In the production of iron in a blast furnace the above reaction is usually completed before the material reaches the high temperature of the fusion zone. To accomplish 45 this reaction in the electric furnace, as heretofore constructed, has been a matter of uncertainty and difficulty; and it is one object of the present invention to furnish conditions whereby the above reaction will be 50 accomplished in the regular order of the descent of the material from the feed hopper to the heat zone. In the first heating-up of an electric furnace of this kind, as the coke, 55 charcoal or other carbonaceous material is brought to incandescence by the resistance it offers to the passage of the current, any oxygen within reach will be absorbed, with the formation of carbonic acid ( $CO_2$ ), which 60 gas in the presence of an excess of incandescent carbon speedily becomes reduced to carbonic-oxid gas ( $CO$ ); one molecule of the carbonic acid becoming two molecules of the carbonic-oxid gas. This latter gas then coming 65 in contact with the oxid of iron, in any

of its oxid forms, at a sufficiently high temperature, absorbs oxygen from the ore, with the reduction of the ore to metal, and the formation of one molecule of carbonic acid for each molecule of carbonic-oxid gas. If 70 the carbonic acid thus formed can again be brought into contact with incandescent carbon, and the resulting carbonic oxid gas again brought into contact with iron ore, the same reactions above described will repeatedly take place; and another object of this invention is to so circulate these two gases as to repeatedly bring the carbonic oxid gas as quickly as practicable after its formation into contact with iron ore in its 80 proximity, and afterward, as soon as possible thereafter, to bring the carbonic acid thereby produced into contact with incandescent carbon, and to repeat the cycle of these reactions until the final gas passes out of the 85 furnace at its top.

Other objects will be set forth in the general description which follows.

Four sheets of drawings accompany this specification as part thereof.

Figures 1 and 2 represent axial vertical sections in different planes through an electric smelting furnace, illustrating the improved smelting process; Fig. 3 is a plan view of the top of the furnace above its top 90 plate, indicating by lines A—B and C—D the planes of Figs. 1 and 2, respectively; Fig. 4 represents a detail side view of one of the stoking screws enlarged from Fig. 2; and Figs. 5, 6 and 7 are diagrams representing the paths of the electric current under different conditions.

Like reference characters indicate like parts in all the figures.

The present improvement in the art of 105 electric smelting is preferably and conveniently carried into effect within and by means of the electric smelting furnace represented by said drawings, and may be described in connection therewith as follows: 110 The furnace so represented is of a stack form; its internal structure, *a*, being built of suitable brick or the like within a metallic shell, *b*, of iron or steel, hereinafter referred to as iron; a layer, *c*, of a suitable non-conductor of electricity, such as asbestos, being interposed between the internal structure *a* and the shell *b* throughout. The top plate, *d*, of the shell *b* and of the furnace is conveniently horizontal, and is provided with 115 feeding hoppers, *e*, *f*, *g* and *h*, best shown in Fig. 4, which are so shaped and so united with each other and with the top plate by braces, stays and angle irons, represented respectively at 1, 2 and 3, as to form a truss by 120 which the subjacent top-plate is stiffened against sagging. The respective hoppers, *e*, *f*, *g* and *h* communicate with the upper ends of flue-shaped passages, *i*, *j*, *k* and *l*, which 125 extend downward within the internal struc- 130

ture *a*; and the hoppers *f* and passages *j*, each of them four in number in the specific construction represented by the drawing, are appropriated to the principal charge of ore, 5 hereinafter referred to as the coarse ore, which is thus divided into several distinct columns. Another set of said hoppers and passages, *g* and *h*, external to said coarse-ore passages, are appropriated to fine ore, which 10 may be of that description which is too fine for reduction in a blast furnace, and which is utilized in this arrangement, not only to feed fine ore into the charge, as hereinafter more particularly set forth, but also and pri- 15 marily to conserve the heat of the furnace by intercepting and utilizing heat that would otherwise escape by radiation and by being conducted outward, and to carry the same back into the working chamber so as to protect the iron shell of the furnace against 20 excessive heat, and to utilize such radiant or outwardly directed heat in the reduction of the ore.

The fine-ore passages *k* are divided into 25 inner and outer passages by hollow walls forming a gas space, *m*, Fig. 2, within each wall, open at bottom and in direct communication with said coarse-ore passages *j* and with the working chamber, *n*, by way of outwardly flaring gas tubes, *o*, hereinafter more particularly described. The outer fine-ore 30 passages, marked *k'*, communicate with the working chamber at their lower ends only and are located peripherally, as shown in Fig. 2, so that the body of fine ore within them may be as cool and as continuous as may be practicable, with reference to intercepting and utilizing outwardly directed heat. The inner fine-ore passages, *k* are pro- 35 vided with baffle plates, *p*, Fig. 2, preferably V-shaped in cross section, and arranged with the apex uppermost so as to retard the flow of the fine ore to a sufficient extent without being subjected to breaking strains, and 40 more particularly to form suitably distributed spaces throughout the body of fine ore. From each of these spaces an opening, *p'*, Fig. 2, extends inward through the wall of the working chamber *n*, and affords a dis- 45 charge for more or less of the fine ore as it reaches that point into the outer edges of the coarse-ore columns, so as to gradually mix the two as they approach the heat zone, and to gradually bring the hottest of the fine ore 50 inward toward the center of the furnace and thus to reduce the need of stoking.

The central hopper *e* and the passage *i* extending vertically therefrom are appropriated to suitable dry carbonaceous material, 55 which may consist wholly or in part of charcoal or coke and is hereinafter referred to as coke. The coke column so formed is intended to preserve its identity from top to bottom of the furnace in the 60 initial charge, and from the top to the fluid

contents of the hearth when the furnace is in operation, as in Figs. 1 and 2. Said coke passage *i* is formed by a central circular wall at the top of the furnace, and this wall is supported by partition walls in the form 70 of flying buttresses, arranged in pairs around said central wall, and forming between them where their inner edges are exposed below said circular wall, a wing-shaped passage, *i'*, Fig. 1, in communication 75 with said central passage *i*, above each of the main electrodes, *q*, *r*, *s*, and *t*, so that the coke may spread laterally in the form of wings between and below said partition walls, and extend the separation of the columns of coarse ore as hereinafter described. The other four of said hoppers, shown at *h* in Figs. 1 and 3, and the peripheral passages, *l*, leading downward therefrom, are appropriated to the feed of resistance regulating 80 material adapted to flow downward by gravity and to protect the main electrodes and regulate the conductivity of the charge at the heat zone as set forth in the previous specification hereinbefore referred to. I 85 still prefer as such material broken electrode carbons reduced to suitable fragments so as to feed by gravity, which insures a regulating material of greater conductivity than the charge of coke or charcoal. Said main electrodes *q*, *r*, *s*, and *t* are preferably four 90 in number and arranged in two pairs at right angles to each other and horizontal as aforesaid. They are located immediately above the hearth, *u*, and each of them in the 95 specific construction shown in the drawings comprises a carbon body, *5*, preferably built up of relatively small carbons, and securely united with ample electric contact to a metallic stem, *6*, preferably of aluminum. Each 100 of these electrode stems extends outward through a water-cooled stuffing box, *7*, which is mounted on a face-plate, *8*, covering an opening through which the body of the electrode may be introduced and withdrawn, 105 and detachably secured to the iron shell *b*. Insulation against the leakage of electricity 110 is introduced between the electrode stem and the gland of the stuffing box, and between the face-plate and iron shell, either or both. 115 Secondary electrodes, *v* and *w*, are located respectively at the bottom and top of the furnace; the bottom electrode, *v*, having a carbon body, *9*, which forms a lining for the hearth *u* of the furnace, and is connected 120 with a depending central metallic stem, *10*. Suitable provision is made for cooling the electrode stem *10*, as indicated by the water circulating pipes 18 and 19, Fig. 1, the details of which may be of any known or improved description. The other electrode stems may obviously be cooled in like manner. Said electrode stem *10* protrudes through a water-cooled stuffing box, *20*, mounted on a face plate, *21*, which is bolted 125 130

to the bottom of the furnace, so as to be detachable, and when detached exposes an opening, 22, through which the end disk 10' of the stem is introduced and withdrawn.

- 5 The secondary electrodes, *w*, at the top of the furnace, are preferably four in number, located above the respective main electrodes *q*, *r*, *s* and *t*. The metallic stem, 27, of each of these electrodes extends upward through 10 a water cooled stuffing box, 28, on the top plate *d* as shown in Figs. 1 and 3. The carbon bodies of the top electrodes *w*, or the top electrodes proper, are supported sub- jacently within rectangular pockets, 29, Fig. 15 1, formed in the walls of the central coke passage *i*, so that the face of the carbon body of each of these electrodes is substantially flush with the inner surface of said wall, and in contact with the charge of coke 20 through which the electric current passes from the bottom electrode *v* to the top electrodes *w*; the latter being of one polarity.

The two sets of electrodes, that is to say the main electrodes, *q*, *r*, *s*, *t*, and the secondary electrodes, *v*, *w*, are preferably connected electrically with different dynamos; and the latter are preferably of the two-phase or alternating type, for the main electrodes, at least. The bottom electrode *v* 25 forms the lining, as aforesaid, of a hearth *u*, which is made of ample capacity and is located immediately beneath the main electrodes *q*, *r*, *s*, and *t*, and provided with an outlet, 30, through which to run off the fluid 30 metal, and an outlet, 31, at a higher point, for molten slag. The hearth portion of the furnace is suspended from an annular metallic sill, 32, which may rest upon columns or the like in customary manner, and the 35 depending portion of the hearth is provided with a water jacket, 23, provided with suitably located inlet and outlet connections, 34 and 35, Fig. 1.

An annular gas chamber, 36, Figs. 1 and 45 2, at the top of the furnace, communicates freely with the coarse-ore and coke passages, and with the intermediate passages for fine ore and regulating material, and discharges through an outlet pipe, 37, Figs. 1 and 3.

50 For circulating the gases within the furnace, with reference to promoting the reduction of oxid iron ore in the manner hereinbefore described, and gas spaces *m* formed within the several fine-ore sections of the 55 furnace, as shown in Fig. 2, communicate as already mentioned with tubes *o*. These tubes *o* extend through the inner fine-ore passages (*k*) from the coarse-ore passages *j*, outward into curbs, 38, which project inward to such gas spaces *m* from outside the furnace; and rotary blowers, 39, in the form of electric fans, are located within the outer ends of said tubes and driven by electric 60 motors, *x*, attached to the iron shell *b* of the furnace; the operation being to draw

through the ore into said gas spaces *m* the carbonic oxid gas,  $\text{CO}$ , formed at and in the vicinity of the heat zone, and to force the resulting carbonic acid,  $\text{CO}_2$ , through the coarse ore into the central column of hot coke, by which it is again reduced to carbonic oxid gas, so as to render possible the repetition of this reaction sufficiently to reduce the fine ore to a considerable extent as it escapes from beneath the baffle plates *p*, 70 through the openings *p'*, on its way to the heat zone and before reaching the hottest part of the furnace. The blower tubes *o* are so located as to keep the blowers *x*—39 from opposing one another.

80 The columns of coarse ore and coke within the working chamber of the furnace are separated initially at top by partitions formed as already indicated by flying buttresses sprung between the wall of the working chamber *n* and the central circular wall within which the top electrodes *w* are located. Compare Figs. 1 and 2. The initial separation of the columns thus insured perpetuates itself downward, within the working chamber *n*; as indicated in Figs. 1 and 2, where the charge of the furnace is represented in the plane of section.

85 The regulating material descending by gravity through its passages *l*, as shown in Fig. 1, tends by its greater weight to feed itself beneath the superjacent wings of the coke column, upon and between the main electrodes, *q*, *r*, *s*, *t*, as shown in this figure; and the several streams may be manipulated, 90 if desired, to increase or lessen their effect in regulating the operation of the furnace, by means of suitable stokers provided with insulated handles and introduced through stoke holes 4, Fig. 1. The fine-ore passages 95 *k*—*k'* and gas spaces *m*, terminate at bottom in open ends within arched recesses, *y*, Fig. 2. The fine ore thus released tends to fall inward to a greater or less extent as indicated in Fig. 2, and any particles which may 100 enter with the gases into the gas spaces *m* are immediately discharged therefrom so as to keep said spaces clear.

105 To insure the inward feed of the ore to a sufficient extent, suitable stoking means are 110 provided beneath the several fine-ore passages *k*. Such means may consist of stoking screws, *z*, Fig. 2 and Fig. 4. The fine ore, descending by gravity to the plane of these stoking screws *z* is there forced inward 115 toward the heat zone, as represented in Fig. 2, carrying with it and intermingling with more or less of the coarse ore. The stoking screws *z* are rotated for this purpose by means of worm gearing, 40, which may be 120 driven by hand cranks or by electric motors. Compare Figs. 2 and 4. The screws *z* have 125 their main bearings in water-cooled stuffing boxes, 41, and outer bearings within yokes, 42, attached to the face plates, 43, which 130

support said stuffing boxes and between which and the iron shell *b* water-cooled frames, 44, and ample insulation are interposed. Each of the screws is also constructed with a section, 45, of insulating material, interposed between the inner portion of the screw and its outer stem, 46, to prevent the passage of the electric current outward through the screws. The screws *z* may be of iron and the insulating sections 45 of any suitable material that will resist the furnace heat as well as the electric currents, as for example a suitable asbestos or asbestos-and-mica compound. The inlet and outlet water connections of each stuffing box 41 and each water-cooled frame 44 are represented respectively in Fig. 4 at 47—48 and 49—50. The openings capped by the face-plates 43 and through which the stoking screws are inserted endwise into the furnace and withdrawn for renewal or repairs are represented at 51 in Fig. 4.

For the purpose of oxidizing fortuitous accumulations of carbon or other oxidizable materials at or in the proximity of the focus of the furnace, the inner and outer stems of the working screws shown at *z* are provided with axial passages, 52, Fig. 4, and the outer stems 46 are connected by swivel couplings, 53, with hose or pipes, 54, through which air or other suitable oxidizing material may be blown into the center of the working chamber *n* at will.

One or more man holes, 57, Fig. 2, suitably capped, and conveniently located beneath one or more of the stoking screws *z*, provide for entering the furnace after it is emptied and cooled for the renewal of repair of the electrodes and other like work, and may also be utilized in arranging the charge preliminarily. In preliminarily charging the furnace, the hearth *u* is filled with coke, and a column of coke is built up within the working chamber *n* surrounded by coarse ore to a sufficient height to insure the completion of a continuous coke column extending from the bottom electrode *v* to a point more or less near the upper ends of the top electrodes *w*. Simultaneously, after the plane of the main electrodes, *q, r, s, t*, is reached, fine ore may be fed in through the fine-ore hoppers, *g*, until the fine-ore passages, *k, k'*, are filled or substantially filled. The passages, *l*, for regulating material, above the several main electrodes, *q, r, s, t*, may be filled at the same time or subsequently, and the streams of regulating material may be suitably directed over and in contact with the main electrodes, as shown in Fig. 1.

The electric current is turned on, first through the secondary electrodes *v* and *w*, as illustrated diagrammatically by Fig. 5, and through the intervening column of coke, which is thus rendered incandescent. The

current is then turned on through the main electrodes, *q, r, s, t*, and its supply to both sets from different dynamos as aforesaid, may be simultaneous as illustrated diagrammatically by Fig. 6. The current may thus be passed through the charge by way of all the electrodes throughout the reducing operation, or the secondary electrodes, *v—w*, may be used only occasionally as required. The height to which the central coke column is kept incandescent may be determined by passing more or less current therethrough by way of said secondary electrodes as required, and that in turn determines the proportion of carbon in the molten metal as it reaches the hearth, and facilitates producing either pig iron or steel at will. The gas circulating blowers, *x*—39, are started as soon as the coke column is incandescent, so as to insure the conversion of the carbon-oxid gas formed in the vicinity of the heat zone into carbonic acid, and the conversion of the latter into carbonic-oxid gas again, and so on alternately as above described. Suitable fluxes are added to the several columns of ore and possibly to the coke, as may be required, and the supply of materials by way of the several hoppers, *e, f, g, h*, at the top of the furnace, is kept up so as to render the operation of the furnace substantially continuous.

Stoking at the stoke holes 4, Fig. 1, is resorted to occasionally as may be required to render the operation of the main electrodes, *q, r, s, t*, substantially uniform; and the stoking screws *z* are operated from time to time as may be required to regulate the feed of the fine ore inward to the heat zone. The fluid metal is run off from time to time or continuously through the tap hole, 30, Fig. 1, and the molten slag through its outlet 31, Fig. 1. The discharge of gas through the pipe 37 at the top of the furnace may be continuous, and may, if desired, be promoted by an exhaust fan; the gas being stored, for use in engines or otherwise, in known or improved ways.

The electric connections may include suitable switches for varying the flow of the current through the main electrodes, *q, r, s, t*, as illustrated by Fig. 12 of said Patent No. 702117, dated June 10, 1902; and in like manner provision may be made for disconnecting the main electrodes from their normal source of supply and throwing them into circuit with the bottom electrode *v*, as illustrated by Fig. 7, in order to melt out the contents of the hearth *u* after temporarily suspending the operation.

Suitable carbonaceous material will in most cases be mixed with the ore, and other mixtures may obviously be fed into the working chamber through the several hoppers at the top of the furnace to produce alloys or otherwise to regulate or vary the product of the furnace. For example, large

- pieces or chunks of electrode carbon may be fed into the central hoppers *e* occasionally or systematically, so as to become parts of the coke column and to feed slowly downward therein, with reference to their accumulation to a sufficient extent between the main electrodes, *q*, *r*, *s*, *t*, to hold back one or more of the materials for reduction, and to insure proper conductivity without obstructing the trickling of streams of the molten metal downward between the electrodes into the hearth.

The electric smelting furnace shown in the drawings accompanying my present specification is more fully described and shown together with modifications thereof in the specification forming part of my application for patent, Serial No. 438115, filed June 12, 1908, hereinbefore referred to and the drawings accompanying the same, and forms no part of the invention hereinafter claimed.

Having thus described said improvement, I claim as my invention, and desire to patent under this specification:

- 25 1. The method of charging an electric smelting furnace of the stack type having horizontal electrodes, which consists in maintaining within the furnace a central column of dry carbonaceous material, feeding material for reduction downward in separate columns at the sides of said central column and in contact therewith, and further separating said columns of material for reduction by feeding carbonaceous material downward between them and in contact therewith above the several electrodes.
- 30 2. The method of charging an electric smelting furnace of the stack type having horizontal electrodes, which consists in maintaining within the furnace a central column of dry carbonaceous material, feeding material for reduction downward in separate columns at the sides of said central column and in contact therewith, and further separating said columns of material for reduction by feeding carbonaceous material downward between them and in contact therewith above the several electrodes, such separating material consisting partly of wings of said central column and partly of streams of harder and heavier resistance regulating material.
- 35 3. The method of charging an electric smelting furnace of the stack type having horizontal electrodes, which consists in maintaining within the furnace a central column of dry carbonaceous material, feeding coarse ore downward in separate columns at the sides of said central column and in contact therewith, simultaneously feeding fine ore downward in separate columns external to said coarse ore columns, and further separating said ore columns by feeding carbonaceous material downward between them above the several electrodes.

4. The method of charging an electric smelting furnace of the stack type having horizontal electrodes, which consists in maintaining within the furnace a central column of dry carbonaceous material, feeding coarse ore downward in separate columns at the sides of said central column and in contact therewith, simultaneously feeding fine ore downward in separate columns external to said coarse ore columns, further separating said ore columns by feeding carbonaceous material downward between them above the several electrodes, and mixing the hottest of the fine ore with the coarse ore on their way to the plane of the electrodes.

5. The method of smelting electrically conductive material in an electric furnace of the stack type having horizontal electrodes, which consists in feeding a column of carbonaceous material downward into the space between the electrodes and wings of said column above the respective electrodes, introducing the material for reduction in connection with suitable fluxes at the sides of said column and wings and feeding the same by gravity within the working chamber in separate columns which descend at the sides of said column and wings and at the sides of said electrodes but sufficiently removed therefrom to prevent the reduction of the material to a short-circuiting mass between the electrodes, and passing a suitable current through the charge by way of said electrodes.

6. The method of smelting electrically conductive material in an electric furnace of the stack type having horizontal electrodes arranged in pairs at right angles to each other, which consists in feeding downward a central column of carbonaceous material between the electrodes and wings of the same above the several electrodes, and feeding downward the material for reduction in columns separated from each other by the carbonaceous material and confined to the several quarters of the furnace, whereby the reduction of the conductive material to a short-circuiting mass between the electrodes is prevented; a suitable current being passed through the charge by way of said electrodes.

7. In the reduction of electrically conductive material by smelting in an electric furnace of the stack type having horizontal electrodes, the method of preventing the formation of a pasty mass between the electrodes and thereby short-circuiting the current, which consists in feeding a column of carbonaceous material downward between said electrodes, and feeding in therewith large pieces of relatively hard and conductive carbonaceous material adapted to bridge the space between the electrodes and hold back the material for reduction.

8. In the reduction of ores by smelting in

- an electric furnace of the stack type having horizontal main electrodes and secondary electrodes at top and bottom, the method of preventing the formation of a pasty mass between the main electrodes and thereby short-circuiting the current, which consists in feeding a column of carbonaceous material downward between said main electrodes, expanding the heat zone upward by way of said column by passing a suitable current through said secondary electrodes, and thus insuring the reduction of ore to metal above said main electrodes.
9. In the reduction of ores by smelting in an electric furnace of the stack type having horizontal main electrodes and secondary electrodes at top and bottom, the method of preventing the formation of a pasty mass between the main electrodes and thereby short-circuiting the current, which consists in feeding a column of carbonaceous material downward between said main electrodes and expanding the heat zone upward by way of said column by passing a suitable current through said secondary electrodes, reducing ore to metal in the form of globules above the plane of said main electrodes, and causing the same to trickle downward between said main electrodes.
10. In the reduction of ores by smelting in an electric furnace of the stack type having horizontal main electrodes and secondary electrodes at top and bottom, the method of preventing the formation of a pasty mass between the main electrodes and thereby short-circuiting the current, which consists in feeding a column of carbonaceous material downward between said main electrodes and expanding the heat zone upward by way of said column by passing a suitable current through said secondary electrodes, superheating the same at this point by a sufficient current passing through said main electrodes, and collecting the metal in superheated condition in a subjacent hearth.
11. In the reduction of ores by smelting in an electric furnace of the stack type having horizontal electrodes, and in which the material for reduction is fed downward within the working chamber in columns by gravity, the method of removing fortuitous accumulations of carbon or other oxidizable material, which consists in the introduction of suitable oxidizing material into the center of the furnace as needed.
12. In the reduction of oxid ores by smelting in an electric furnace of the stack type having horizontal main electrodes immediately above its hearth and secondary electrodes at the top of the furnace, the process which consists in maintaining a gravity fed central column of carbonaceous material contacting with said top electrodes and extending downward therefrom, feeding the ore downward by gravity at the sides of said column of carbonaceous material and in communication therewith and passing suitable currents of electricity through the charge by way of said main electrodes, and through said column of carbonaceous material by way of said secondary electrodes.
13. In the reduction of oxid ores by smelting in an electric furnace of the stack type having electrodes at top and bottom, the process which consists in maintaining within the furnace a gravity fed central column of carbonaceous material which forms a resistance conductor between said top and bottom electrodes, feeding the ore downward by gravity at the sides of said column of carbonaceous material and in communication therewith, passing a suitable current of electricity through said electrodes and said column, producing carbonic oxide gas by reducing said column of carbonaceous material to incandescence, bringing said gas into contact with contiguous ore continuously for its reduction to metal, and passing the resulting carbonic acid continuously into contact with the incandescent column of carbonaceous material.
14. In the reduction of oxid ores by smelting in an electric furnace of the stack type having horizontal main electrodes and secondary electrodes at top and bottom, the process which consists in maintaining a gravity-fed central column of carbonaceous material which forms a resistance conductor between said top and bottom electrodes, feeding the ore downward by gravity at the sides of said column of carbonaceous material, passing suitable currents of electricity through said main electrodes and said secondary electrodes respectively, producing carbonic oxide gas by reducing said column of carbonaceous material to incandescence, bringing said gas into contact with contiguous ore for its reduction to metal, and afterward as quickly as practicable passing the resulting carbonic acid into contact with the incandescent column of carbonaceous material again.
15. In the reduction of oxid ores by smelting in an electric furnace of the stack type having horizontal main electrodes and secondary electrodes at top and bottom, the process which consists in maintaining a gravity-fed central column of carbonaceous material which forms a resistance conductor between said top and bottom electrodes, feeding the ore downward by gravity at the sides of said column of carbonaceous material, passing suitable currents through said main electrodes and said secondary electrodes respectively, producing carbonic oxide gas by reducing said column of carbonaceous

- material to incandescence, bringing said gas into contact with contiguous ore for its reduction to metal, afterward as quickly as practicable passing the resulting carbonic acid into contact with the incandescent column of carbonaceous material again, repeating the cycle of these reactions, and discharging the final gas at the top of the furnace.
- 10 16. In the reduction of sesquioxid of iron to metal by smelting in an electric furnace of the stack type having horizontal main electrodes and secondary electrodes at top and bottom, the process which consists in feeding the sesquioxid and suitable carbonaceous material downward by gravity, passing a suitable current through said secondary electrodes to render the column of carbonaceous material incandescent and thereby producing carbonic oxid gas, bringing said gas into contact with the sesquioxid for its reduction into metal above the plane of said main electrodes, afterward as quickly as practicable passing the resulting carbonic acid into contact with the incandescent carbonaceous material again, and superheating the metal as it trickles downward between said main electrodes into the hearth of the furnace.
- 15 17. In the reduction of ore by smelting in an electric furnace of the stack type having horizontal main electrodes arranged in two pairs at right angles to each other and secondary electrodes at top and bottom, the process which consists in maintaining a gravity-fed central column of carbonaceous material forming a resistance conductor between said secondary electrodes and passing a suitable current therethrough, feeding the material for reduction downward by gravity at the sides of said central column, and passing a two-phase current through the charge by way of said main electrodes.
- 20 18. In the reduction of ore by smelting in an electric furnace of the stack type having horizontal main electrodes and secondary electrodes at top and bottom, the process which consists in maintaining a gravity-fed central column of carbonaceous material forming a resistance conductor between said secondary electrodes and passing a suitable current therethrough, feeding the material for reduction downward by gravity at the sides of said central column and in communication therewith, passing a two-phase cur-

rent through the charge by way of said main electrodes, reducing the ore to metal above the plane of said main electrodes, superheating the same as it trickles downward between the main electrodes into the hearth of the furnace, and discharging the fluid metal.

19. In the reduction of ore by smelting in an electric furnace of the stack type having horizontal main electrodes and secondary electrodes at top and bottom, the process which consists in feeding downward by gravity a central column of carbonaceous material forming a resistance conductor between said secondary electrodes, feeding the ore downward by gravity at the sides of said central column and in communication therewith, passing a suitable current through said central column by way of said secondary electrodes to start the operation and to render said column incandescent to a sufficient height, maintaining sufficient heat by passing suitable currents through the charge by way of said main electrodes, and running off the fluid metal from the subjacent hearth.

20. In the reduction of ore by smelting in an electric furnace of the stack type having horizontal main electrodes and secondary electrodes at top and bottom, the process which consists in feeding downward by gravity a central column of carbonaceous material forming a resistance conductor between said secondary electrodes, feeding the ore downward by gravity at the sides of said central column and in communication therewith, passing a suitable current through said central column by way of said secondary electrodes to start the operation and to render said column incandescent to a sufficient height, maintaining sufficient heat by passing suitable currents through the charge by way of said main electrodes, causing carbonic oxid gas from said incandescent column to flow continuously into the ore and carbonic acid from the ore to flow continuously into the incandescent column for conversion into carbonic oxid, discharging the gaseous by-product at the top of the furnace, and running off the fluid metal from the subjacent hearth.

EDWARD R. TAYLOR.

Witnesses:

C. N. MCFARREN,  
S. McDONALD.